

Jan. 1, 1952

E. L. HALL

2,580,767

PROCESS FOR MANUFACTURING OIL GAS

Filed Oct. 1, 1948

2 SHEETS—SHEET 1



FIG. I

INVENTOR  
EDWIN L. HALL  
BY HIS ATTORNEYS

*Houston & Houston*

Jan. 1, 1952

E. L. HALL

2,580,767

PROCESS FOR MANUFACTURING OIL GAS

Filed Oct. 1, 1948

2 SHEETS—SHEET 2



INVENTOR

EDWIN L. HALL

BY HIS ATTORNEYS

FIG. 2

*Houzeon &  
Houzeon*

Patented Jan. 1, 1952

2,580,767

# UNITED STATES PATENT OFFICE

2,580,767

## PROCESS FOR MANUFACTURING OIL GAS

Edwin L. Hall, Cleveland Heights, Ohio, assignor  
to American Gas Association, Incorporated,  
New York, N. Y., a corporation of New York

Application October 1, 1948, Serial No. 52,284

6 Claims. (Cl. 48—214)

1

The present invention relates to a novel process for the manufacture of oil gas, and more particularly it relates to an improved process for the manufacture of oil gas by the pyrolysis of petroleum oils in a regenerative-heating operation.

Oil gas has been manufactured for many years by procedures in which petroleum oil is vaporized and pyrolyzed; in the presence of a gaseous diluent such as steam, in zones of stored heat. A zone, or zones, is first heated by burning a fuel and passing the hot products of combustion of the burning fuel therethrough, and, when the zones are sufficiently heated, oil is then vaporized and, in the presence of a gaseous diluent, pyrolyzed into fixed gases by abstracting heat stored in the zone. After a gas making run, the zone is again heated, followed by another gas making run, and so on. This method of heating is referred to as cyclic heating as contrasted, for example, to the vaporization of oil in a still where heat is applied continuously to the oil directly from the heat source. In order to pyrolyze the vaporized oil properly not only must the vaporized oil be cracked into molecular fragments, but the cracked materials must be held in a heated zone for a sufficient time for the gaseous system to reach equilibrium during which time the highly reactive molecular fragments become converted into stable molecules of gaseous compounds. To bring this conversion about, the cracked vaporized oil is swept from the initial vaporizing and cracking zone, which is at a relatively high temperature, through a path of stored heat, or "fixing zone." The temperatures in the fixing zone must be controlled so that the average temperature thereof is relatively low as compared to that of the combustion-vaporizing zone where vaporization and initial cracking of the oil takes place, with the highest temperature adjacent the combustion-vaporizing zone and with the temperatures progressively decreasing toward the exit end. By the time the vapors have reached the relatively cooler exit end of this zone, the gas has been fixed and it may then be cooled with the removal of condensable constituents.

In the present commercial process, for instance, there is provided a combustion-vaporizing zone, which is often merely the carburetor-generator cell of a carbureted water gas system; and a path of stored heat, or fixing zone, which is often the "superheater" of the carbureted water gas system. The combustion-vaporizing zone is merely a chamber providing a space, surrounded by high temperature-resisting walls of heat-conducting material, wherein fuel, such as tar, gas or oil, and air are forced in the proper ratio for combustion, and burned. The hot products of combustion heat the walls of the chamber, and are swept through the "superheater" where heat is stored in a checkerwork of ceramic material, and thence out the stack. This step is referred to as the "blow." Then oil and steam are ad-

2

mitted to the combustion-vaporizing zone where the oil is vaporized and cracked, and the mixture is swept through the hot checkerwork where it is fixed into permanent gas, and thence to the wash box. As indicated above, the step is referred to as the "gas making run" or simply as the "make." These steps are repeated continuously as long as required for the gas-making operation. Generally, the apparatus is "purged" with air or steam between the "blow" and the "make," or between the "make" and the "blow," or both, to remove undesirable products, to recover the gas remaining in the system and to prevent the accumulation of explosive mixtures. There are various modifications of the commercial process as outlined above, all of which, however, are based on the same sequence of steps.

There are limitations imposed by the above set forth procedure which are becoming presently more serious. As indicated previously, the optimum conditions throughout the system embody a combustion-vaporizing zone of relatively high temperature, followed by a fixing zone of relatively low average temperature as compared to that of the combustion-vaporizing zone and in which the temperature progressively decreases toward the exit end. These conditions are met in present day processes only with difficulty since the temperature throughout the system depends for the most part upon the combustion of oil during the "blow," and a rate of combustion adapted to provide a relatively high temperature in the combustion-vaporizing zone similarly results in undesirably high temperatures in the subsequent path. In other words, the top temperature limit in the combustion-vaporizing zone is restricted in order to provide the necessary temperature conditions in the fixing zone. As a result, the temperature in the combustion-vaporizing zone cannot be maintained as high as desirable on the one hand, and the temperature of the fixing zone cannot be maintained as low as desired on the other, and thus a relatively wide temperature gradient between the combustion-vaporizing zone and the exit end of the fixing zone, which would represent the optimum conditions, cannot be obtained economically in present day procedures. This is further aggravated by the fact that the steam admitted into the combustion-vaporizing zone during the gas making run has a cooling effect on that portion of the apparatus which it is desired to have at the highest temperature.

Moreover, the present commercial processes can only satisfactorily utilize low residual carbon oils in the gas-making run. For instance, oils containing over 6-7% free carbon, as determined by the Conradson test more fully described hereinafter, cannot be employed successfully in the gas-making run because of the fact that the carbon deposited on the checkerwork in that por-

tion of the fixing zone which is adjacent the combustion-vaporizing zone, will in time clog the system. It has thus been necessary to employ only the low residual carbon oils which are relatively expensive as compared to the more abundant oils containing higher quantities of Conradson carbon, or high residuum oils. A method of manufacturing oil gas wherein high carbon oils may be utilized as the gas-making oil is becoming increasingly desirable with the advent and increasing use of catalytic and thermal cracking techniques in the petroleum refining industry which result in more highly cracked residuum oils which produce much higher ratios of carbon upon gasification. The economies of the gas industry require the successful use of the cheapest residual oils that the petroleum industry provides. Furthermore, even the carbon deposited in the checkerwork during present commercial oil gas operations represents a waste since it cannot be utilized in the system but must be removed by periodic cleaning or by intermittent blasts of air or steam.

All these mentioned limitations, of course, combine to seriously limit the capacity of the apparatus during the gas-making run. That is to say, since the temperature of the combustion-vaporizing zone, on the one hand, cannot be maintained as high as desired, less efficient fuel combustion than is possible is obtained during the blow; and since the temperatures in the fixing zone, on the other hand, cannot be maintained as low as desired, less efficient gasification is obtained during the gas-making run due to overcracking. Furthermore, since carbon deposited is removed by unduly long "blow" periods, further inefficiency is encountered. Thus, there is room for improvement in the presently practiced procedures with the aim of overcoming the limitations set forth above.

It is, therefore, a principal object of the present invention to provide an economical process for the manufacture of oil gas whereby the aforementioned disadvantages are for the most part overcome or eliminated.

Another object is to provide a process for the manufacturer of oil gas wherein there is readily established between the combustion-vaporizing zone and the fixing zone, temperature gradients favorable to the production of the maximum quantity of high heat unit gas per unit of gas-making oil employed.

Another object is to provide a process whereby steam employed in the gas-making run may be preheated to a high temperature prior to the admission to the combustion-vaporizing zone of a gas-making unit while at the same time insuring optimum temperature gradients during the process.

A specific object is to provide a process for the manufacture of oil gas whereby heavy residuum and high Conradson carbon oils may be readily employed as gas-making oils.

A specific object is to provide a process for the manufacture of oil gas whereby greater efficiency is obtained by the utilization of the carbon deposited in the system during preceding gas-making runs as a part of the fuel required in the subsequent storage of heat in the system.

A further object is to provide a process for the manufacture of oil gas whereby heat losses due to the loss of sensible heat in the made gas is kept at a minimum.

Further objects, including the provision of a novel apparatus in which to conduct the process,

will be apparent from a consideration of the following specification and claims.

In accordance with the present invention, there is provided a continuous regenerative process for the manufacture of oil gas by the pyrolysis of petroleum oils in which heat is stored in two independently heated interconnected paths of stored heat, each of which is preceded by a combustion-vaporizing zone in flow communication therewith, which comprises admitting fluid fuel and air into the combustion-vaporizing zone preceding one of said paths; burning said fuel in said combustion-vaporizing zone, the products of said burning being swept along said path to store heat therein, abstracting a portion of said heat from the other of said paths of stored heat by passing, in the direction of its communicating combustion - vaporizing zone, steam therethrough to superheat said steam; admitting said superheated steam to the first mentioned combustion-vaporizing zone concurrently with the admission of petroleum oil thereto; vaporizing and pyrolyzing said petroleum oil in the presence of said steam in said first mentioned combustion-vaporizing zone and in said first mentioned path; withdrawing said vaporized and pyrolyzed oil and said steam from said first mentioned path; and repeating said sequence of steps with a reversal of the order of said two paths of stored heat.

It will be noted from the above that in accordance with the broader aspects of the present process there are provided a pair of gas-making units, each unit comprising, in flow communication, a combustion-vaporizing zone and a gas-fixing zone. The sequence of steps that occur, i. e. "blow" and "gas-making run" in each unit are roughly the same as that occurring in present day procedures, with the exception that steam introduced into the combustion-vaporizing zone of one of the units during the gas-making run is previously preheated to a high temperature by passing it through the fixing zone and combustion-vaporizing zone of the other unit from the exit end of the former in the direction of the latter. This exception, however, provides many unexpected advantages as well as fulfilling a part of the objects outlined above. In the first place, by passing steam through one unit in the direction stated preparatory to its admission to the other for its gas-making step, a wider temperature gradient is provided in the first unit preparing it for its subsequent heating and gas-making runs. In other words, the temperature of the fixing zone of the first unit is materially reduced from a point adjacent to its communicating combustion-vaporizing zone outwardly towards its exit end so that during its subsequent "blow" or heating step greater combustion can be had in its communicating combustion-vaporizing zone with consequent higher temperatures therein, while still maintaining a relatively low mean temperature in the fixing zone, with the temperatures in the fixing zone progressively decreasing toward the exit end. In the second place, while performing this valuable function, the steam also becomes heated to a high temperature obviating the use of auxiliary steam-heaters. This also eliminates the cooling effect encountered in prior procedures when the heat in the combustion-vaporizing zone was relied upon to superheat the steam.

Preferably, however, heat is also abstracted from the fixing zone of one unit by passing air

therethrough from the exit end thereof in the direction of and through its communicating-combustion-vaporizing zone. The hot gases thus leaving that combustion-vaporizing zone are admitted to the combustion-vaporizing zone preceding the other path concurrently with the admission of a fluid fuel thereto during the "blow" or heating step. This feature, along with the superheating of the steam during the gas-making run as above described, combine to form a particularly valuable commercial process. Thus, in accordance with the preferred process of the present invention, a portion of the stored heat from one of said independently heated, interconnected paths of stored heat is abstracted by passing air therethrough in the direction of its communicating combustion-vaporizing zone to raise the temperature of the air and to burn carbon in said path and its communicating combustion-vaporizing zone. The resulting hot gases are then admitted to the combustion-vaporizing zone preceding the other of said paths concurrently with the addition of fluid fuel thereto. The fuel is burned in the presence of said hot gases in said combustion-vaporizing zone, the products of said burning being swept through the path communicating therewith to store heat therein. A further portion of stored heat is then abstracted from the first mentioned path of stored heat by passing steam therethrough in the direction of, and through, its communicating combustion-vaporizing zone to superheat the steam, and the superheated steam is admitted to said combustion-vaporizing zone preceding said second mentioned path concurrently with the addition of petroleum oil thereto. The petroleum oil is vaporized and pyrolyzed in the presence of said superheated steam in the said combustion-vaporizing zone and in the said second mentioned path of stored heat, and the vaporized and pyrolyzed oil and steam are withdrawn from said path. The cycle is completed by repeating the above sequence of steps with a reversal of the order of said two paths of stored heat. A gas-making process of the same general type in which air is passed countercurrently through one unit preparatory to its admission to the other as described, but in which steam, if used, is not preheated in the manner described above, forms the subject matter of copending application, Serial Number 52,283, filed October 1, 1948.

Thus, in accordance with the preferred embodiment as outlined above, the passage of the air and the steam through one unit in the direction stated preparatory to their admission to the other unit during the respective "blow" and "gas-making" steps results in a greater temperature gradient between the combustion-vaporizing zone and fixing zone of each unit than is the case when only steam is preheated in the manner described preparatory to the gas-making runs. Of equal importance, however, is the fact that the air passing through one unit in the direction stated becomes progressively hotter as it approaches the point in the apparatus where carbon deposited from the preceding gas-making run is heaviest. The hot air causes combustion of carbon in this unit not only removing it but further raising the temperature of the resulting gaseous mixture to a high degree just prior to its admission into the combustion-vaporizing zone of the other unit. This not only eliminates cooling, due to the admission of cool air into the combustion-vaporizing zone of the

other unit, but also provides more efficient combustion of the oil therein. Furthermore, since the hot mixture of gases entering the combustion-vaporizing zone contains a relatively large amount of sensible heat, both due to the abstraction of heat from the first unit and due to the combustion of carbon deposited therein, a correspondingly less amount of fuel is required for the "blow," or heating step, in the second unit. The reduction in the amount of fuel required increases with the amount of carbon deposited by the gas-making oil which is in turn burned during the passage in the manner described of the air through the unit containing the deposited carbon. Thus in accordance with the preferred embodiment not only can less expensive oil be employed in the gas-making run, but the cheaper the grade employed, i. e. the higher the quantity of carbon it deposits during cracking, the smaller the quantity of fuel required.

It will be also noted from the above that the high temperatures are concentrated in that portion of each unit where they are most necessary, i. e. in the combustion-vaporizing zones, and that portion of the fixing zone immediately adjacent each combustion-vaporizing zone; while lower temperatures are provided where they are most desirable, i. e. in the fixing zone with temperatures progressively decreasing toward the exit end thereof. The net result of this is that more efficient combustion of fuel is obtained in each combustion-vaporizing zone during the particular "blow" or heating step of that unit, and more efficient gasification with less over-cracking is obtained in each unit during its particular gas-making run.

The present invention may be more readily understood by a consideration of the drawings in which Figure 1 illustrates the main steps of a complete cycle of the present process, and Figure 2 illustrates the main steps of a complete cycle of the preferred embodiment of the invention.

Referring more particularly to the drawings, Figure 1, as stated, illustrates the main steps of the invention. There are shown in Figure 1 two oil-gas-making units 10 and 11 each of which is provided with a combustion-vaporizing zone 14 and 15, respectively, and a path of stored heat, i. e. fixing zone, 12 and 13, respectively. While, for the sake of description, distinct combustion-vaporizing zones and distinct fixing zones are shown in the drawings, it will be understood that often, in actual practice, no clear boundary line between the combustion-vaporizing zone and its communicating fixing zone can be fixed. As seen in 1<sup>a</sup>, which illustrates the heating step for unit 11, there are means for selectively introducing steam into the exit end of each unit. One method of doing this is shown in 1<sup>a</sup> wherein conduits leading to the exit ends of each unit 10 and 11 are connected to a common source of steam by means of two way valve 17. By this arrangement steam may be directed to either of the units as desired or turned off completely. The succeeding steps shown in drawings, 1<sup>b</sup>, 1<sup>c</sup> and 1<sup>d</sup>, which illustrate the gas-making step in unit 11, the heating step for unit 10, and the gas-making step in unit 10, respectively, show the directions of flow of the steam, or, if no flow direction is shown, the fact that no steam is flowing in that step. Similarly 1<sup>a</sup> shows means for selectively withdrawing the materials from the respective units. One method of doing this is shown in 1<sup>a</sup> by providing appropriate conduits

leading from the exit end of each unit 10 and 11 to a conventional two-way valve 18, so that the gas coming from the respective units may be directed to the wash box as required. As shown in 1<sup>a</sup> conventional conduits leading to a stack are also provided. In this case also, the succeeding steps as seen in 1<sup>b</sup>, 1<sup>c</sup> and 1<sup>d</sup> show the direction of flow from the respective units. There are, of course, conduit means interconnecting both combustion-vaporizing zones, and in 1<sup>b</sup> and 1<sup>d</sup> the direction of flow through these means during the various steps is indicated. Since, for the purposes of the broader aspects of the present invention as illustrated in Figure 1, gas-making unit 11 may be idle during unit 10 heating step as shown in 1<sup>c</sup>, the representation of unit 11 in 1<sup>c</sup> has been omitted.

While each gas-making unit is illustrated in the figure as a unitary structure, it will be understood that the combustion-vaporizing zone of each may be a separate structure or cell, such as a conventional generator-carburetor unit of the type used in present day oil-gas, or carbureted water-gas industries, each of which is in flow communication with a separate fixing zone such as a conventional "superheater" of the type employed in present day oil-gas or carbureted water-gas industries. Since the figure illustrates the main steps of a complete cycle, it is understood that the system has already been heated to start the process, as is conventional, by burning fluid fuel such as oil, tar or gas in each combustion-vaporizing zone and blasting the hot combustion gases through the respective fixing zones. Units 10 and 11 may be connected to a common stack or, as is preferred, to separate stacks in order to avoid "hot" valves, and may be connected either to a common wash box, or to separate wash boxes. Although combustion-vaporizing zones 14 and 15 have been, for the purpose of description, illustrated as separate structure, it will be understood that, since the conduit means interconnecting them is large so as to handle the hot gases, combustion-vaporizing zones 14 and 15 and the interconnecting conduit means may be developed in practice into a single chamber.

As shown in 1<sup>a</sup> of Figure 1, the cycle may be started, after each unit has been heated to the extent desired for starting the process as is well known in the art, by admitting air and a fluid fuel to the combustion-vaporizing zone of one of the units, in this case, combustion-vaporizing zone 15 of unit 11. The fuel is burned in combustion-vaporizing zone 15 and the hot combustion-products are swept through the fixing zone 13, and thence out the stack.

The next main step is shown in 1<sup>b</sup> where steam is passed through unit 10 from the exit end thereof through fixing zone 12 and combustion-vaporizing zone 14, respectively. As the steam passes through unit 10 it abstracts heat from fixing zone 12 which has been stored therein by a previous "blow" step. As the steam approaches combustion-vaporizing zone 14 it becomes progressively hotter. However, due to its initial cooling effect upon its admission to the exit end of unit 10, the temperature throughout unit 10 progressively decreases from the combustion-vaporizing zone 14 outwardly toward the exit end. The passage of steam in the direction stated thus tends to concentrate high temperatures where they are required, i. e. in combustion-vaporizing zone 14 and in that portion of the fixing zone 12 which is adjacent to the combustion-vaporizing zone 14, while at the same time providing a relatively

wide temperature gradient between the combustion-vaporizing zone 14 and the exit end of the fixing zone 12. The highly superheated steam leaving unit 10 is then admitted to combustion-vaporizing zone 15 of unit 11, substantially concurrently with the admission of gas-making oil thereto. In combustion-vaporizing zone 15 the oil is vaporized, and substantial cracking of the vaporized oil takes place. Because of the large amount of sensible heat contained in the superheated steam, the steam serves as a heating medium for the vaporized oil and also as heat transfer medium between the hot surfaces in unit 11 and the vaporized oil. It will also be realized that gas-making oil may be admitted to combustion-vaporizing zone 14 while the steam is passing therethrough, in which case it is also admitted to combustion-vaporizing zone 15 concurrently with the superheated steam.

The thus vaporized and pyrolyzed oil and the steam are then passed through fixing zone 13 where the more reactive molecular fragments of cracked gas become converted to stable gaseous molecules. However, since steam has previously been passed through unit 11 in the same manner as in unit 10 as above-described, a wider temperature gradient is provided in the same manner as was described above with respect to unit 10. Thus the average temperature in fixing zone 13 is lower than that in conventional fixing zones facilitating the "fixing" of the gas therein and decreasing to a marked extent the danger of over-cracking. The fixed gas and steam leaving fixing zone 13 from the exit end thereof and directed to a wash box.

1<sup>c</sup> and 1<sup>d</sup> illustrate the completion of the cycle by a repetition of the above steps with, however, a reversal in the order of units. As shown in 1<sup>c</sup> air and a fluid fuel are admitted to combustion-vaporizing zone 14 of unit 10. As in 1<sup>a</sup> the fuel is burned and the hot combustion products are swept through fixing zone 12 storing heat therein. However, since unit 10 has just previously been swept with steam, as described above and as illustrated in 1<sup>b</sup>, the higher temperatures are concentrated in combustion-vaporizing zone 14 and in that portion of the fixing zone 12 which is adjacent thereto; while the temperatures in the fixing zone 12 progressively decrease toward its exit end. The next main step, as shown in 1<sup>d</sup> corresponds to that shown in 1<sup>b</sup>, except the order is reversed. Steam is passed through fixing zone 13 of unit 11 toward, and through, combustion-vaporizing zone 15. The passing steam abstracts heat stored during the preceding "blow" as shown in 1<sup>a</sup>, with the greatest cooling effect being produced near the exit end, and with the concentration of the highest temperatures at and near the combustion-vaporizing zone 15. The thus superheated steam is admitted to combustion-vaporizing zone 14 of unit 10 concurrently with the addition of gas-making petroleum oil thereto. As described above zone gas-making oil may also be admitted to combustion-vaporizing zone 15 as the steam is passing therethrough. In unit 10 the oil is vaporized and pyrolyzed in the same manner as described previously with respect to 1<sup>b</sup>, and the fixed gas leaves the exit end of fixing zone 12, going to the wash box.

The gas produced in each unit may then be treated by procedures which are well known in the gas-making industry, by being subjected to conventional cooling and condensing operations. Normally, the hot gas is fed to a wash box which is merely the primary condenser where the gas

is cooled to below the boiling point of water, and condensable constituents such as tar and other hydrocarbons are removed. As stated above, a common wash box advantageously may be employed having a capacity adapted to receive the products from both units.

As indicated above, Figure 1 shows the main steps of the process and it will be understood that suitable "purges" may be, and advantageously are conducted between one or more of the various steps. For instance, between the steps set forth as 1<sup>a</sup> and 1<sup>b</sup> and between 1<sup>c</sup> and 1<sup>d</sup>, a blast of air is advantageously swept through in the direction shown without introducing heating oil into the respective combustion-vaporizing zones. This removes from the system undesirable products formed by the combustion of the fuel before the gas-making run is begun. Similarly, between the steps illustrated as 1<sup>b</sup> and 1<sup>c</sup> and between steps 1<sup>d</sup> and 1<sup>a</sup>, a blast of steam is advantageously swept through the respective units in the direction shown to clear the system of oil-gas. In this purging step, there is also advantageously a blast of steam admitted from the exit end of the unit in which oil gas has just been made to insure that no explosive mixtures of gas and air will be obtained when the subsequent "blow," or heating step is performed.

Figure 2, as stated, illustrates the main steps of the preferred embodiment of the present invention. As in Figure 1, there are shown in Figure 2 two oil gas-making units 20 and 21 each of which is provided with a combustion-vaporizing zone, i. e., 24 and 25, respectively, and a path of stored heat, or "fixing zone," i. e., 22 and 23, respectively. As previously pointed out, while each gas-making unit is illustrated in the figure as a unitary structure, it will be understood that the combustion-vaporizing zone of each unit may be a separate structure or cell each of which is in flow communication with a separate fixing zone. As also pointed out above, while for the sake of description, distinct combustion-vaporizing zones and distinct fixing zones are shown in the drawings, it will be understood that often, in actual practice, no clear boundary line between the combustion-vaporizing zone and its communicating fixing zone can be fixed. Since the figure illustrates the main steps of a complete cycle, it is to be understood that the system has been already heated to start the process, as is conventional, by burning fluid fuel in each combustion-vaporizing zone and blasting the hot combustion gases through the respective fixing zones. Units 20 and 21 may be connected to a common stack or, as is preferred, to separate stacks, in order to avoid "hot" valves, and may be connected either to a common wash box, or to separate wash boxes.

As shown in 2<sup>a</sup>, which illustrates the heating step for unit 21, the cycle may be started, after each unit has been heated, by passing air through one of the units, in this case unit 20, from the exit end thereof, i. e. the end from which the made oil-gas leaves the unit, through the fixing zone 22 and the combustion-vaporizing zone 24, respectively. During its passage the air becomes progressively hotter and at the same time cools the fixing zone 22 somewhat, by abstracting a portion of the heat stored therein. The hot air causes carbon deposited in combustion-vaporizing zone 24, and in that portion of fixing zone 22 which is adjacent combustion-vaporizing zone 24 to burn. Deposited carbon in fixing zone 22 and combustion-vaporizing zone 24 is not only thus removed but also serves as

part of the fuel necessary for supplying heat to combustion-vaporizing zone 24 and to unit 21. The resulting hot mixture of gases is then admitted to combustion-vaporizing zone 25 of unit 21 concurrently with the addition of a fluid fuel thereto. Because of the large amount of sensible heat contained in the hot gases entering combustion-vaporizing zone 25, less fuel is required to supply heat to unit 21, and that which is burned is burned more efficiently. Additional air, supplementing any admitted from unit 20, may be supplied to combustion-vaporizing zone 25 if necessary. The combustion products from combustion-vaporizing zone 25 are swept through fixing zone 23, storing heat therein. However, since unit 21 has just previously been swept successively with air as described above, and with steam as will be described below, relatively large amounts of heat, with correspondingly high temperatures, are concentrated in combustion-vaporizing zone 25 and in that portion of fixing zone 23 adjacent combustion-vaporizing zone 25, while the temperatures in fixing zone 23, rapidly decrease toward its exit end. The combustion products leaving fixing zone 23 may be directed to a stack where they are discarded.

The next main step, that is the gas-making step in unit 21, is shown in 2<sup>b</sup> where steam is passed through unit 20 in the same manner as has been described with respect to 1<sup>b</sup> in Figure 1. The steam passing through fixing zone 22 abstracts a further portion of heat stored therein. During its passage through fixing zone 22 the steam becomes progressively hotter until by the time it reaches combustion-vaporizing zone 24 relatively little heat is abstracted by the hot steam. As has been pointed out above with respect to Figure 1, some gas-making oil may be admitted into the passing steam at this point in combustion-vaporizing zone 24. Nevertheless, due to its initial cooling effect the temperatures near the exit end of fixing zone 22 will be further lowered, resulting in even a greater temperature gradient between the two ends of the unit. The thus superheated steam is then admitted to combustion-vaporizing zone 25 of unit 21 concurrently with the admission of gas-making oil thereto. In combustion-vaporizing zone 25 vaporization and substantial cracking of the oil takes place. The mixture of cracked gas and steam then flows through fixing zone 23 in which its resides for sufficient time for the cracked gas to become converted to stable gaseous molecules. The fixed gas, and steam, are then directed to a wash box.

Figures 2<sup>c</sup> and 2<sup>d</sup>, which illustrate respectively the heating step for unit 20 and the gas-making step in unit 20, show a repetition of the steps outlined above with, however, a reversal of the order of units. As shown in 2<sup>c</sup>, air is passed through fixing zone 23 and combustion-vaporizing zone 25. As in the previously described steps, carbon deposited during the preceding gas-making run, is burned and the hot mixture of gases is admitted to combustion-vaporizing zone 24 concurrently with the admission of fluid fuel thereto. The fuel is burned in the presence of the hot gases and the hot combustion products are swept through fixing zone 22, storing heat therein, and thence to a stack. As illustrated in 2<sup>d</sup> steam is then passed countercurrently through unit 21, as was described above with respect to 2<sup>b</sup>, and the thus superheated steam and gas-making oil are admitted concurrently to combustion-vaporizing zone 24 of unit 20. As has been described previously some gas-making oil may be admitted to

combustion-vaporizing zone 25 as the steam is passing therethrough, in which case it also enters combustion-vaporizing zone 24 concurrently with the steam. In combustion-vaporizing zone 24 the oil is vaporized and cracked, and the vaporized and cracked material is passed through fixing zone 22 as described previously. The fixed gases leaving unit 20 are directed to a wash box. The process as illustrated in Figure 2 is continued, of course, by repeating the cycle beginning with the steps shown in 2<sup>a</sup>.

As indicated above, Figure 2 shows the main steps of the preferred process and it will be understood that suitable "purges" may be, and advantageously are conducted between one or more of the various steps. For instance, between the steps set forth as 2<sup>a</sup> and 2<sup>b</sup> and between 2<sup>c</sup> and 2<sup>d</sup>, a blast of air is advantageously swept through the respective units in the direction shown without introducing heating fuel into the respective combustion-vaporizing zones. This removes from the system undesirable products formed by the combustion of the fuel before the gas-making run is begun. Similarly, between the steps illustrated as 2<sup>b</sup> and 2<sup>c</sup> and between steps shown in 2<sup>c</sup> and 2<sup>d</sup>, a blast of steam is advantageously swept through the respective units in the direction shown to clear the system of oil-gas. In this purging step, there is also advantageously a blast of steam admitted from the exit end of the unit in which oil-gas has just been made to insure that no explosive mixtures of air and gas will be obtained when the subsequent "blow," or heating step is performed.

As also seen in 2<sup>a</sup> there are means for selectively introducing steam or air into the exit end of each unit. One method of doing this is shown in 2<sup>a</sup> wherein conduits leading to the exit ends of each unit 10 and 11 are connected, through two-way valves 27 and 28, respectively, to sources of steam and air. By this arrangement steam may be directed to either of the units as desired or turned off completely, or air may be directed to either of the units as desired or turned off completely. The succeeding steps shown in drawings 2<sup>b</sup>, 2<sup>c</sup> and 2<sup>d</sup> show the directions of flow of steam or air as the case may be. Similarly 2<sup>a</sup> shows means for selectively withdrawing the materials from the respective units. One method of doing this, as shown in 2<sup>a</sup>, is by providing conventional conduits leading from the exit end of each unit 10 and 11 to a two-way valve 26 so that the gas coming from the respective units may be directed to a wash box as required. As also shown in 2<sup>a</sup> conventional conduits leading to a stack are provided. In this case also, the succeeding steps, as seen in 2<sup>b</sup>, 2<sup>c</sup> and 2<sup>d</sup> show the direction of flow of materials from the exit ends of the respective units. There is, of course, as is also the case in Figure 1, conduit means interconnecting the combustion-vaporizing zone of each unit. In 2<sup>a</sup>, 2<sup>b</sup>, 2<sup>c</sup> and 2<sup>d</sup> the direction of flow through this conduit means is indicated.

Referring to the apparatus that may be employed, each part, i. e. the combustion-vaporizing zone and the fixing zone, may be those presently employed in the gas-making industry. As indicated above, the combustion-vaporizing zone may be any of the well known structures used for that purpose, such as the carburetor section of the conventional carbureted water gas apparatus, or one of the combined generator-carburetor structures of conventional oil-gas systems. Specifically, the combustion-vaporizing zone is merely a chamber of heat-conducting material,

which is capable of resisting high temperatures, such as clay fire brick, carborundum brick, and the like, designed for the combustion of the fluid heating fuel, and, after it has become sufficiently heated, for the vaporization of the gas-making oil. The walls of the chamber ordinarily provide sufficient area to store the heat required for the subsequent vaporization and initial cracking of the gas-making oil. The chamber may be completely empty, or may have a portion thereof equipped with checkerwork of ceramic material, such as clay, fire brick, carborundum brick, and the like, in which sensible heat may be stored.

As is customary in present day oil gas-making procedures, the combustion-vaporizing zone is provided with a burner adapted to handle the particular fuel employed. Normally, the burner is essentially a jet or jets which inject the fuel into the combustion-vaporizing zone. The burner may be provided with means to mix incoming air with the fuel before it is injected into the combustion-vaporizing zone, or some or all of the air may be separately admitted into the combustion-vaporizing zone. In any event, air and fuel are admitted to the combustion-vaporizing zones in the ratios providing efficient combustion of the fluid fuel. The combustion-vaporizing zones are also equipped with means for injecting the gas-making oil thereinto. Such means are well known in the gas-making industry and generally comprise a nozzle or nozzles adapted to spray the oil into the zone at the appropriate time.

With respect to air passed through one unit preparatory to its admission to the other unit during the heating steps, at least sufficient air is passed through the first unit to burn the carbon therein. If the air passed through the first unit is just sufficient to burn carbon therein, supplementary air may be added to the combustion-vaporizing zone wherein combustion of fluid fuel is taking place in an amount to support combustion of the fuel. On the other hand, air in excess of that required for burning the deposited carbon may be passed through the first unit, in which case the amount of supplemental air required is correspondingly decreased. Thus, the amount of air passed through the first unit may be sufficient not only to burn carbon deposited therein but also to support the combustion of at least the major portion, and even all of the fluid fuel admitted to the combustion-vaporizing zones.

With respect to the path of stored heat or "fixing zone" it may be any of those structures which are well known and are used for that or similar purposes in the oil-gas, or carbureted water-gas, industry. It is essentially a large chamber of high temperature-resisting material such as fire brick, the inside of which is provided with many passage ways through which the gaseous material must flow. Customarily, the inside is provided with a checkerwork of high temperature-resisting material such as clay brick with the portion of checkerwork which is to be subjected to the highest temperatures, i. e. that portion which is nearest the combustion-vaporizing zone, being made of carborundum brick. The fixing zone is of sufficient volume to permit the passing gases to reside there until converted or "fixed" into stable commercial oil-gas. The exact size and shape of the fixing zone will be dictated by the considerations well known in the gas-making industry, including capacity desired, requisite holding time, and the like.

Referring to the fuel employed during the "blow" or heating step for storing heat in each unit, as indicated previously, it may be any of the fluid fuels ordinarily employed in the gas-making industry such as petroleum oil, tar, gas, and the like. Generally, the fuel employed will be a petroleum oil and a wide variety of such oils are available for this use such as Numbers 2 and 3 furnace oils, heavy residuum oils, and the like. As stated, tar, such as coal tar, carbureted water gas tar, and oil gas tar such as is obtained in the process, may also be used as the fuel, in which case it will possess sufficient fluidity to be handled by the burner and injected into the combustion-vaporizing zone. The proper fluidity may be obtained in some cases by heating the tar, or heavy oil if used, or by thinning them with less viscous miscible liquids of the same nature, or by a combination of these means.

As indicated above, the preferred process permits the utilization of a wide range of gas-making petroleum oils. Whereas previous processes were restricted to the use of petroleum oils containing less than 7%, and preferably less than 4% Conradson carbon, the present preferred process is readily adapted for the utilization of petroleum oils containing as high as 13% Conradson carbon or even higher. (Conradson carbon is the proportion of carbonaceous residue remaining after a standardized heating cycle is performed on a weighed quantity of the particular oil following the procedure set forth under the A. S. T. M. designation D189-36. In accordance with that procedure, a weighed quantity of oil is heated at a predetermined rate in a crucible until a cokelike residue is left, and this residue is then heated to red heat. From the weight of the carbon remaining, the Conradson carbon content of that oil is calculated as the percentage thereof based on the weight of the oil sample employed.) In any event, any of those petroleum oils heretofore used such as gas oil or diesel oil or lighter hydrocarbons, for example, kerosene, gasoline, liquefied petroleum gases, such as propane, butane and the like, may be employed, and, when the preferred process is practiced, petroleum oils which have heretofore been unusable such as those containing more than about 7% Conradson carbon, may be used.

In accordance with the present process steam which has been superheated as described, is introduced into the combustion-vaporizing zone concurrently with the gas-making oil in order to reduce the partial pressures of the oil vapors. The relative proportions of superheated steam and gas-making oil may vary widely as is well known in the art. For example, the proportion of steam to gas-making oil may range from about 1 part of the former to 1 of the latter, by weight, to about 1 part of the former to about 10 parts of the latter by weight.

The average temperatures in each unit will be similar to those employed during conventional procedures, for example, between about 1150° F. and about 2000° F. and preferably between about 1400° F. and about 1650° F. However, it will be realized that due to the novel procedure herein set forth, relatively higher temperatures, e. g. 100° F. to 500° F. higher, than heretofore will be concentrated at the combustion-vaporizing zones of each unit, while the temperature near the exit end of each fixing zone will be somewhat lower, e. g. 100° F. to 500° F. lower, than those employed in conventional processes.

The following examples illustrate the opera-

tion of the process and are not intended to limit the scope of the invention in any way.

#### EXAMPLE I

- 5 Two gas-making units were set up, each of which comprised a combustion-vaporizing zone and a fixing zone. Prior to the gas-making run in each unit, steam was superheated in the other as described herein, and prior to the "blow" in each unit air was passed through the other unit, as also described herein. The test lasted 22.58 hours during which time there were about 170 cycles. Each cycle lasted 8 minutes. The combined "blow" periods consumed about 51% of each cycle, and the combined "make" periods consumed about 39% of each cycle. Purges and valve action accounted for the remaining time in each cycle.
- 10 The oil employed, both as gas-making oil and as fuel oil was a petroleum oil having a Conradson carbon content of 0.2%. Unit #1 used 2260 gallons of fuel oil, and unit #2 consumed 3313 gallons, indicating a total consumption of fuel oil amounting to 1.01 gallons per thousand cubic
- 15 feet of gas made. Unit #1 consumed 32,981, gallons of gas-making oil, and unit #2 consumed 33,342 gallons, indicating a total consumption of gas-making oil mounting to 11.98 gallons per thousand cubic feet of gas made, and a total
- 20 consumption of oil, both fuel and gas-making, of 12.98 gallons per thousand cubic feet of gas.

The average temperatures during the operation were as follows:

|                                  | °F.  |
|----------------------------------|------|
| 35 Combustion-vaporizing zone #1 | 1740 |
| Bottom of fixing zone #1         | 1665 |
| Top of fixing zone #1            | 1370 |
| Combustion-vaporizing zone #2    | 1440 |
| Bottom of fixing zone #2         | 1690 |
| 40 Top of fixing zone #2         | 1090 |

Steam was employed during the "make" at the rate of 68 lbs. per minute, and air was preheated during the "blow" at the rate of 15,538 cubic feet per minute. Supplemental air was introduced at each combustion-vaporizing zone during each "blow" at the rate of 11,737 cubic feet per minute.

The gas made mounted to 5,538,000 cubic feet, and possessed a heat unit content, as determined by a calorimeter, of 1042 B. t. u. per cubic foot.

#### EXAMPLE II

The same procedure was followed as in Example I with the exception that a petroleum oil with a Conradson carbon content of 6.02% was employed as fuel oil and gas-making oil.

|                                   |                         |
|-----------------------------------|-------------------------|
| Time of operation                 | 17 hours                |
| Time of each cycle                | 8 minutes               |
| Time consumed in "blow"           | 48%                     |
| Time consumed in "make"           | 43%                     |
| 60 Gallons fuel oil consumed:     |                         |
| Unit #1                           | 1,885 gals.             |
| Unit #2                           | 1,867 gals.             |
| Volume of gas made                | 4,294 MCF <sup>1</sup>  |
| Heating value of gas              | 1017 B. t. u./cu. ft.   |
| Gallons fuel oil consumed/MCF gas | .87 gals./MCF           |
| Gallons gas-making oil consumed:  |                         |
| Unit #1                           | 23,018 gals.            |
| Unit #2                           | 23,180 gals.            |
| Gallons gas-making oil/MCF gas    | 10.76 gals./MCF         |
| Gallons total oil used/MCF gas    | 11.63 gals./MCF         |
| Average temperatures:             |                         |
| Combustion-vaporizing zone #1     | 1570° F.                |
| Bottom of fixing zone #1          | 1600° F.                |
| Top of fixing zone #1             | 1290° F.                |
| Combustion-vaporizing zone #2     | 1430° F.                |
| Bottom of fixing zone #2          | 159° F.                 |
| Top of fixing zone #2             | 1040° F.                |
| 70 Steam rate during "make"       | 100 lbs. per minute     |
| Air rate during "blow":           |                         |
| Preheated                         | 16,536 cu. ft. per min. |
| Supplemental                      | 11,596 cu. ft. per min. |

<sup>1</sup> MCF=Thousand cubic feet.

**15**  
**EXAMPLE III**

The same procedure was followed as in the foregoing examples with the exception that a petroleum oil having a Conradson carbon content of 13.03% was used as fuel oil and as gas-making oil.

|                                      |                      |
|--------------------------------------|----------------------|
| Time of operation                    | 24 hours             |
| Time of each cycle                   | 8 minutes            |
| Time consumed in "blow"              | 42%                  |
| Time consumed in "make"              | 49%                  |
| Gallons fuel oil consumed:           |                      |
| Unit #1                              | 465 gals.            |
| Unit #2                              | 435 gals.            |
| Volume of gas made                   | 3779 MCF             |
| Heating value of gas                 | 976 B. t. u./cu. ft. |
| Gallons of fuel oil consumed/MCF gas | .24 gal.             |
| Gallons gas-making oil consumed:     |                      |
| Unit #1                              | 21,299 gals.         |
| Unit #2                              | 21,517 gals.         |
| Gallons gas-making oil/MCF gas       | 11.33/MCF            |
| Gallons total oil used/MCF gas       | 11.57/MCF            |
| Average temperatures:                |                      |
| Combustion-vaporizing zone #1        | 1540° F.             |
| Bottom of fixing zone #1             | 1595° F.             |
| Top of fixing zone #1                | 1355° F.             |
| Combustion-vaporizing zone #2        | 1460° F.             |
| Bottom of fixing zone #2             | 1600° F.             |
| Top of fixing zone #2                | 1030° F.             |
| Steam rate during "make"             | 129 lbs./minute      |
| Air rate during "blow":              |                      |
| Preheated                            | 15,586 cu. ft./min.  |
| Supplemental                         | 9,396 cu. ft./min.   |

The advantages of the present process will be more readily appreciated by a consideration of the following table. In the table, data collected from tests similar to those set forth in the examples were converted to the basis of 1,000 cu. ft. of 1000 B. t. u. gas. Four different oils were employed, in group A, a 0.2% Conradson carbon oil was used; in group B a 3% Conradson carbon oil was used; in group C a 6% Conradson carbon oil was used, and in group D is a 13% Conradson carbon oil was used. In each group, with the exception of group D, performance data obtained as the result of the present process listed as the odd numbered tests, are compared with data obtained as the result of a conventional gas-making procedure listed as even-numbered tests. Since group D employed 13% Conradson carbon oils, the apparatus of the conventional procedure became clogged and no data could be collected.

*Table I*

| Group | Test | Gals. fuel oil/MCF <sup>1</sup> | Gals. make oil/MCF | Gals. total oil/MCF | MCF gas per hour | Thermal Efficiency <sup>2</sup> |
|-------|------|---------------------------------|--------------------|---------------------|------------------|---------------------------------|
| A     | 1    | .90                             | 11.50              | 12.49               | 248              | 78.6                            |
|       | 2    | 1.60                            | 11.42              | 13.11               | 200              | 75.3                            |
| B     | 3    | .79                             | 11.40              | 12.19               | 213              | 80.4                            |
|       | 4    | .98                             | 12.55              | 13.53               | 140              | 74.5                            |
| C     | 5    | .94                             | 10.88              | 11.52               | 206              | 81.2                            |
|       | 6    | .90                             | 12.43              | 13.33               | 138              | 76.9                            |
| D     | 7    | .28                             | 11.60              | 11.97               | 149              | 80.9                            |
|       | 8    |                                 |                    |                     |                  |                                 |

<sup>1</sup> Thousand cubic feet of gas.  
<sup>2</sup> Heat units in gas and tar based on heat units in starting oil.

Considerable modification is possible in the variation of details in practicing the process of the present invention without departing from the scope thereof.

I claim:

1. The process for the manufacture of oil gas by the pyrolysis of petroleum oil in which heat is stored in each of two gas-making units, each of which gas-making unit comprises a fixing zone in flow-communication with a combustion-vaporizing zone, the combustion-vaporizing zones of said two gas-making units being in flow-communication with each other, which comprises introducing air into the combustion-vaporizing zone of one of said units while burning fluid fuel therein, the resulting hot gaseous products being swept through its communicating fixing zone

**16**

to store heat therein; abstracting a portion of the heat stored in the fixing zone and in the combustion-vaporizing zone of the other of said gas-making units by passing steam through said fixing zone in the direction of its communicating combustion-vaporizing zone and thence through said combustion-vaporizing zone to superheat said steam; admitting said superheated steam to the combustion-vaporizing zone of the said first-mentioned unit concurrently with the admission of petroleum oil thereto; vaporizing and pyrolyzing said petroleum oil in the presence of said superheated steam in the combustion-vaporizing zone and fixing zone of said first-mentioned unit; withdrawing the vaporized and pyrolyzed oil and steam from said first-mentioned unit; then introducing air into the combustion-vaporizing zone of said second-mentioned unit while burning fluid fuel therein, the resulting hot gaseous products being swept through its communicating fixing zone to store heat therein; abstracting a portion of the heat stored in the fixing zone and the combustion-vaporizing zone of said first-mentioned unit by passing steam through said fixing zone in the direction of its communicating combustion-vaporizing zone and thence through said combustion-vaporizing zone to superheat said steam; admitting said superheated steam to the combustion-vaporizing zone of the said second-mentioned unit concurrently with the admission of petroleum oil thereto; vaporizing and pyrolyzing said petroleum oil in the presence of said superheated steam in the combustion-vaporizing zone and fixing zone of said second-mentioned unit; withdrawing the vaporized and pyrolyzed oil and steam from said second-mentioned unit, and repeating cyclically said sequence of steps.

2. The process of claim 1 wherein the fluid fuel is petroleum oil.
3. The process of claim 1 wherein the fluid fuel is tar.
4. The process for the manufacture of oil gas by the pyrolysis of petroleum oil in which heat

is stored in each of two gas-making units, each of which gas-making units comprises a fixing zone in flow-communication with a combustion-vaporizing zone, the combustion-vaporizing zones of said two gas-making units being in flow-communication with each other, which comprises abstracting a portion of said stored heat from the fixing zone and combustion-vaporizing zone of one of said units by passing air through said fixing zone in the direction of its communicating combustion-vaporizing zone and thence through said combustion-vaporizing zone of said first-mentioned unit; admitting the resulting hot gases to the combustion-vaporizing zone of the other of said units while burning fluid fuel therein, the resulting hot gaseous products being swept through the fixing zone of said second-

mentioned unit to store heat therein; abstracting a further portion of heat from the fixing zone and combustion-vaporizing zone of said first-mentioned unit by passing steam through said fixing zone in the direction of its communicating combustion-vaporizing zone, and thence through said combustion-vaporizing zone, to superheat said steam; admitting said superheated steam to the combustion-vaporizing zone of said second-mentioned unit concurrently with the admission of petroleum oil thereto; vaporizing and pyrolyzing said petroleum oil in the presence of said superheated steam in the combustion-vaporizing zone and fixing zone of said second-mentioned unit; withdrawing said vaporized and pyrolyzed oil and said steam from said second-mentioned unit; then abstracting a portion of said stored heat from the fixing zone and combustion-vaporizing zone of said second-mentioned unit by passing air through said fixing zone in the direction of its communicating combustion-vaporizing zone and thence through said combustion-vaporizing zone, to raise the temperature of said air and to burn carbon in said fixing zone and said communicating combustion-vaporizing zone of said second-mentioned unit; admitting the resulting hot gases to the combustion-vaporizing zone of said first-mentioned unit while burning fluid fuel therein, the resulting hot gaseous products being swept through the fixing zone of said first-mentioned unit to store heat therein; abstracting a further portion of heat

from the fixing zone and combustion-vaporizing zone of said second-mentioned unit by passing steam through said fixing zone in the direction of its communicating combustion-vaporizing zone, and thence through said combustion-vaporizing zone, to superheat said steam; admitting said superheated steam to the combustion-vaporizing zone of said first-mentioned unit concurrently with the admission of petroleum oil thereto; vaporizing and pyrolyzing said petroleum oil in the presence of said superheated steam in the combustion-vaporizing zone and fixing zone of said first-mentioned unit; withdrawing said vaporized and pyrolyzed oil and said steam from said first-mentioned unit, and repeating cyclically said sequence of steps.

5. The process of claim 4, wherein the fluid fuel is petroleum oil.

6. The process of claim 4, wherein the fluid fuel is tar.

EDWIN L. HALL.

#### REFERENCES CITED

25 The following references are of record in the file of this patent:

#### UNITED STATES PATENTS

| Number    | Name           | Date           |
|-----------|----------------|----------------|
| 2,174,196 | Rogers         | Sept. 26, 1939 |
| 2,192,815 | Johnson et al. | Mar. 5, 1940   |
| 2,208,123 | Duncan         | July 16, 1940  |